

Patented Feb. 9, 1926.

1,572,502

# UNITED STATES PATENT OFFICE.

ALADAR PACZ, OF CLEVELAND, OHIO, ASSIGNOR, BY MESNE ASSIGNMENTS, TO  
ALUMINUM COMPANY OF AMERICA, A CORPORATION OF PENNSYLVANIA.

## ALUMINUM ALLOY.

No Drawing.

Application filed September 12, 1919. Serial No. 323,850.

To all whom it may concern:

Be it known that I, ALADAR PACZ, a citizen of the United States, residing at Cleveland, in the county of Cuyahoga and State 5 of Ohio, have invented a new and useful Aluminum Alloy, of which the following is a specification.

My invention relates to improvements in alloys and more particularly alloys of 10 aluminum.

The object of my invention is to provide an alloy which will have a close grained structure and which will therefore, have a very smooth surface when machined, and to 15 provide an alloy possessing to a high degree the properties of resistance to warping when heated, hardness, high tensile strength and resistance to wear. More specifically, the object of my invention is to produce an 20 aluminum alloy which may be used to advantage as a substitute for cast iron which has the disadvantage that it is heavy and can not be machined to present a very smooth surface.

One of the important uses to which my invention may be put is as a material for molds and cores for the manufacture of rubber goods. It is highly desirable to have a metal 25 for this purpose which will be light and therefore easy to handle and still will resist warping when heated. Moreover, it is important that the metal be smooth so that the rubber may be stripped easily therefrom. The high heat conductivity which is 30 possessed by my alloy is also advantageous in this connection as it results in the saving of time. The strength of my alloy is attested by the fact that I have made ring-shaped molds therefrom which have resisted 35 even greater compression than ordinary cast iron molds.

Another important use of my alloy is for cylinders and piston rings for automobile and other engines. The lightness and the 40 comparatively high resistance to wear are of advantage in this connection and the fact that my alloy possesses a certain amount of elasticity is of especial importance in the use of piston rings. It has been proposed to 45 line or cover aluminum parts with material such as iron or steel to obtain a better wearing surface than can be obtained from aluminum but still retaining the advantage of the latter's low specific gravity. My alloy 50 may be used for this purpose and it has the

advantage that its co-efficient of expansion is closer to that of aluminum than that of iron or steel.

While attempts have been made heretofore to substitute aluminum for cast iron as a 60 material for molds for rubber goods such as tires, the best result secured was the production of a comparatively few tires in a single mold. By the use of my alloy, I have been able to produce 120 tires in a single 65 mold without any apparent damage to the core.

Still another use for which my invention may be applied is to articles in which the matter of ornamentation is an important 70 consideration. My alloy possesses a very high lustre, its brilliancy being similar to that of speculum. As my alloy has a low melting point and is very fluid when melted, it is a good material for use in die casting 75 and in general in the manufacture of articles in permanent molds. By varying the composition and if desired, the addition of small percentages of other metals, the color or tone may be varied to suit various tastes. 80

I have produced an alloy which had a sclerometer hardness of 45 while cast iron usually runs between 28 and 40. This material had a tensile strength of 21,000 to 85 24,000 pounds per square inch which compares favorably with cast iron. The specific gravity of the alloy was less than half of that of cast iron.

The alloys embraced by my invention contain copper and silicon. Slight amounts of 90 other metals may be present without appreciable deleterious effect and small percentages of such metals may be added to enhance certain properties which may be desirable for a particular purpose. An alloy in which 95 such additions are incorporated would come within the scope of my invention. It has been heretofore proposed to make alloys of aluminum, copper and silicon but in these cases the silicon was used in a very low 100 amount or, indeed, was present only as an impurity. I have found that with an aluminum content of 70 parts by weight, very good results were secured with the copper varying from 15 to 27½ parts and the silicon from 2½ to 15 parts.

I have obtained exceptionally good results from an alloy of 105 67½ parts aluminum, 25 parts copper and 7½ parts silicon and in another case from 110 an alloy of 72 parts aluminum, 23.5 parts

copper and 4.5 parts silicon. Stated generally, the alloy should consist of at least 50 per cent aluminum and at least  $2\frac{1}{2}$  per cent silicon, the balance being copper. It is preferred however, to keep the copper below 25 per cent.

To produce my alloy I may melt together the copper, aluminum and silicon metals in any suitable manner. I may also 10 produce the alloy from aluminum and copper silicide and I may also use aluminum silicide and copper silicide. These materials are obtainable commercially.

What I claim and desire to secure by Letters Patent of the United States is:—

1. An alloy consisting of aluminum, copper and silicon in the proportion substan-

tially of 70 parts by weight of aluminum, to 15 to  $27\frac{1}{2}$  parts of copper and  $2\frac{1}{2}$  to 15 parts of silicon.

2. An alloy consisting of aluminum, copper and silicon, the aluminum constituting at least 50 per cent by weight, the silicon constituting at least  $2\frac{1}{2}$  per cent by weight and the copper constituting an appreciable percentage by weight.

3. An alloy consisting of aluminum, copper and silicon, the aluminum constituting at least 50 per cent by weight, the copper constituting at least 15 per cent by weight and the silicon at least  $2\frac{1}{2}$  per cent by weight.

ALADAR PACZ.